

## UNITED STATES PATENT OFFICE.

WILLIAM H. BUELL, OF BRONXVILLE, NEW YORK, ASSIGNEE, BY MESNE ASSIGNMENTS, TO CONVERSION PRODUCTS CORPORATION, A CORPORATION OF DELAWARE.

## COATING COMPOSITION FOR METALS AND METHOD OF MAKING SAME.

No Drawing.

Application filed April 12, 1920. Serial No. 373,348.

*To all whom it may concern:*

- Be it known that I, WILLIAM H. BUELL, a citizen of the United States, residing at Bronxville, in the county of Westchester, State of New York, have made a certain new and useful Invention in Coating Compositions for Metals and Methods of Making Same, of which the following is a specification.
- 10 This invention relates to a composition for coating metals or ferrous material, which is especially adapted to prevent the rust of the material, or other deterioration due to oxidation.
- 15 A further object to be mentioned is to provide a method for manufacturing the product.

20 A further object to be mentioned is to provide a composition of the character referred to which is not injurious and is to an extent preservative.

The further objects of the invention will appear more fully hereafter.

25 The invention consists substantially in the process hereinafter set forth, together with the composition formed by the ingredients, all of which will be more fully hereinafter described.

30 It is among the special purposes of my present invention, as hereinbefore outlined, to provide a composition of a greasy character to coat metals and particularly ferrous material such as finely polished steel surfaces, machine tools, automobiles, guns, etc., which will prevent the material from rusting in storage. Many compositions such as vaseline, heavy oils, waxes, greases, etc., have been made heretofore and the great difficulty encountered has been that such 35 compositions have either melted and run off of the material to which they were applied when the material has been subjected to ordinary heat of storage, thereby causing the compositions to lose every effective coating function and allow the material to which they were applied to rust, or were of such character that they could not be easily removed. It has therefore also been among the special purposes of my invention to provide a composition of this character which 40 will not run when subjected to excessive heat and heats of a degree far in excess of normal climatic or natural heats, and which at the same time will permit the ready re-

moval thereof from the material when desired.

To form the composition of my invention, I use the following ingredients in the manner hereinafter set forth, but I wish it to be understood that while I specify particular ingredients as a specific example, together with approximate proportions or percentages thereof employed in the production of the product, I do not desire to be limited or restricted either to the specific ingredients or to the percentages set forth as like ingredients, that is, ingredients having similar characteristics and varied percentages may be employed without departing from the spirit and scope of my invention, as defined in the claims.

As an example, I take ten per cent of aluminum soap of cocoanut oil and thoroughly dissolve the same in thirty per cent of paraffine oil under heat. I then add ten per cent of paraffine and melt the paraffine in the solution, to which is then added fifty per cent of petrolatum. Unless the aluminum soap of cocoanut oil is thoroughly dissolved and mixed with the paraffine oil, the results obtained are not as effective as they otherwise would be.

I have found that it is advantageous to add to the composition obtained as hereinbefore stated, one per cent by weight of an alkali such as a caustic potash solution for the purpose of neutralizing any acid condition in the ingredients of the composition due to impurity or other cause, and to neutralize any acid condition on the surface of the material to which the composition is to be applied. While I do not desire to be limited or restricted in this respect, I find it satisfactory to employ for the alkali a caustic potash solution, consisting of caustic potash dissolved in an alcohol such as methyl alcohol, amyl alcohol, etc., it being readily apparent that the alcohol evaporates, leaving the caustic potash in a free state in the composition. I have found that in addition to the composition produced as hereinbefore set forth being an effective coating composition for metals and particularly ferrous materials to prevent the rusting thereof, that the composition will not run off of the material to which it has been applied, even when the material is subjected to heat as high as 200 degrees Fahrenheit. If rust

- retardation is further desired, there may be added to the composition, for example, a small portion of potassium chromate, or five per cent of a soda or potash soap in addition. 5
- As above stated, I do not desire to be limited or restricted to the specific example herein given, and it is desired that the same be regarded in an illustrative sense rather than in a limiting sense. 10
- Having now set forth, however, the objects and nature of my invention, and having given a specific example thereof, what I claim as new and useful and of my own invention and desire to secure by Letters Patent, is:—
1. The process of manufacturing a rust preventing coating composition, comprising dissolving and thoroughly mixing a metallic soap of a saponifiable oil in an oil, and then adding petrolatum thereto. 15
  2. The process of manufacturing a coating composition comprising dissolving and thoroughly mixing a metallic soap of a saponifiable oil in a solution of a hydrocarbon oil, adding petrolatum to form a solution, and then adding a rust retardant to the solution obtained. 20
  3. The process of manufacturing a coating composition, comprising dissolving and thoroughly mixing a metallic soap of a saponifiable oil in a solution of hydrocarbon, then adding petrolatum thereto, and finally incorporating in said solution an alkali and a rust retardant. 25
  4. The process of manufacturing a coating composition comprising dissolving and thoroughly mixing a metallic soap of a saponifiable oil in a solution of a hydrocarbon, in the presence of heat of a degree above the melting point of the said hydrocarbon and then adding a rust retardant to the solution obtained. 30
  5. The process of manufacturing a coating composition, comprising dissolving and thoroughly mixing a metallic soap of a saponifiable oil in a solution of a hydrocarbon, in the presence of heat of a degree above the melting point of the said hydrocarbon and then adding an alkali to the solution obtained and finally adding an additional rust retardant chemical. 35
  6. The process of manufacturing a coating composition, comprising dissolving and thoroughly mixing aluminum soap of cocoanut oil in a hydrocarbon oil. 40
  7. The process of manufacturing a coating composition, comprising dissolving and thoroughly mixing aluminum soap of cocoanut oil in paraffine oil, then incorporating paraffine, petrolatum and rust retardants. 45
  8. The process of manufacturing a coat- 50
- ing composition, comprising dissolving and thoroughly mixing aluminum soap of cocoanut oil in paraffine oil, then incorporating paraffine, petrolatum, and caustic potash. 65
9. The process of manufacturing a coating composition, comprising dissolving and thoroughly mixing aluminum soap of cocoanut oil in paraffine oil, then adding melted paraffine and then adding petrolatum thereto, then adding a solution of caustic potash, and finally adding a rust retardant chemical. 70
10. The process of manufacturing a coating composition, comprising dissolving and thoroughly mixing aluminum soap of cocoanut oil in paraffine oil, then adding petrolatum thereto, then adding a solution of caustic potash, and finally adding potassium chromate. 75
11. The process of manufacturing a coating composition, comprising dissolving and thoroughly mixing aluminum soap of cocoanut oil in paraffine oil, then adding melted paraffine and then adding petrolatum thereto, then adding a solution of caustic potash, and finally adding potassium chromate. 80
12. A coating composition comprising a composition of aluminum soap of cocoanut oil, paraffine oil, and petrolatum, and caustic potash. 85
13. A coating composition comprising a composition of aluminum soap of cocoanut oil, paraffine oil, petrolatum and potassium chromate. 90
14. A protective coating consisting of a composition of aluminum soap of cocoanut oil, paraffine oil, paraffine, petrolatum, caustic potash, and potassium chromate. 95
15. A protective coating comprising a composition of aluminum soap of cocoanut oil, paraffine oil, paraffine, petrolatum, and potash soap containing free alkali and a chromate. 100
16. The process of manufacturing a coating composition, comprising dissolving and thoroughly mixing aluminum soap of cocoanut oil in paraffine oil, then adding melted paraffine and then adding petrolatum thereto, then adding an alkali to the solution obtained, and finally adding a chromate. 105
17. The process of manufacturing a coating composition, comprising dissolving and thoroughly mixing aluminum soap of cocoanut oil in paraffine oil, then adding melted paraffine and then adding petrolatum thereto, then adding an alkali to the solution obtained, and finally adding potassium chromate. 110
- In testimony whereof I have hereunto set my hand on this 8th day of April A. D., 1920. 115
- WILLIAM H. BUELL.